

Nov. 11, 1952

**R. J. GRIMM**

2,617,743

## METHOD OF MAKING COATED PAPER MOISTURE RESISTANT

Filed March 8, 1952



*INVENTOR.*

RICHARD J. GRIMM.  
BY

BY  
ward, Crosby & Neal

ATTORNEYS.

## UNITED STATES PATENT OFFICE

2,617,743

METHOD OF MAKING COATED PAPER  
MOISTURE RESISTANTRichard J. Grimm, Whitesboro, N. Y., assignor to  
St. Regis Paper Company, New York, N. Y., a  
corporation of New York

Application March 8, 1952, Serial No. 275,605

3 Claims. (Cl. 117—64)

1

This invention relates to methods for manufacturing moisture resistant paper, the invention being particularly adapted, among other possibilities, for the production of relatively inexpensive coated paper adapted for high speed lithographic printing.

In lithographic printing the plate rolls used are ordinarily kept in clean condition by aqueous mixtures, with the consequence that small amounts of moisture, along with the ink, are carried onto the paper during printing. With this method of printing, particularly if coated paper is used and is travelling at a high speed (for example 800—900 feet per minute), such moisture is sufficient to cause particles of the coating to be released and displaced or "picked" off, thus seriously interfering with good quality printing, unless the paper coating is in some way made moisture-resistant.

To provide such moisture-resistance, it has heretofore been common practice to coat the paper "off the machine," that is, as a separate operation after the paper leaves the paper making machine. In such cases casein-clay coating mixtures have been commonly used incorporating an ingredient such as formaldehyde which has the property of rendering water resistant such adhesives as casein. Since with such off-the-machine coating, the speed of the paper during the coating operation is relatively slow, the coating composition used may comprise a quite thin mixture; that is, a mixture of low viscosity and having a high water content, and hence sufficient amounts of formaldehyde solution may be incorporated therein without causing the coating mixture to harden before it is properly applied or distributed on the paper as a coating. However, this method of producing a moisture-resistant paper for the purpose has the disadvantage that the coating of the paper relatively slowly as an operation separate from the manufacture of paper, involves a substantial extra expense as compared with the cost of modern high-speed methods of coating paper on the paper making machine. Accordingly efforts have heretofore been made to provide some way by which paper could be coated on the paper making machine, or without an extra handling operation, to provide a product sufficiently moisture-resistant for high-speed lithographic printing purposes, and with avoidance of the extra cost of off-the-machine coating which may amount to 50% or more. To this end attempts have been made to incorporate in the coating mixture on the paper making machine materials such as formaldehyde or other ingredients for

2

rendering the coating moisture-proof. However, since coating paper at the necessary high speeds on the machine requires the use of a mixture having a high solids content so that it will quickly dry, it has been found that attempts to introduce formaldehyde into such a mixture caused the coating material to more or less solidify so rapidly that it could not be properly applied and uniformly distributed on the paper as a coating. Attempts to use other chemicals for the purpose during coating on the paper machine have not, so far as is known, met with any substantial commercial success, for various reasons.

Other attempts to solve the problem have involved coating the paper on the machine and then the application of a waterproofing agent such as formaldehyde in aqueous solution to the coated paper as it passes over the calender at the end of the paper machine. Still other attempts have involved the application of formaldehyde as a gas to the paper after coating. These attempts also, so far as is known, have not met with any substantial commercial success and involve difficulties of securing uniform treatment throughout the surface of the paper, and also the very serious difficulty that formaldehyde, as an obnoxious gas, escapes into the room to such a serious extent that it cannot be tolerated by the workmen.

According to the present invention, paper is coated by known methods preferably at high speed on the paper making machine by applying thereto known or conventional coating mixtures embodying a pigment such as clay and a proteinaceous adhesive such as casein (or a proteinaceous adhesive such as "isolated soya protein" as commonly used in paper coating mixtures), and then as the paper leaves the dryer rolls of the paper making machine and is about to pass through the machine calender stack, or later as it is about to be passed through the usual supercalender, it is treated with formaldehyde by incorporating the formaldehyde in the so-called "steam showers," such as are customarily used for applying steam to the paper on supercalenders. According to the preferred method, an aqueous solution (containing for example from 10—40% of formaldehyde) is allowed to drip into the hot interior of the steam shower enclosure so that formaldehyde gas is entrained in the streams of steam which are projected through small exhaust apertures onto the paper just as the paper is to pass between the rolls of the calender. Thus the customary steam showers which are used to soften the paper and the coating thereon at the calender, serve forcefully to apply the formaldehyde, caus-

ing it effectively to penetrate the web surface and impart the desired moisture-proof characteristics to the adhesive thereof, and since the application of the formaldehyde in this way is immediately followed by the compressing and smoothing of the paper between the calender rolls, the method has the effect of insuring thorough penetration of the adhesive by the formaldehyde and the prompt locking, in effect, of the formaldehyde into the surface of the web. At the same time it has been found that this method of projecting the formaldehyde as embodied in expanding jets of steam onto the paper is surprisingly effective in preventing objectionable escape of the obnoxious gas into the atmosphere of the room.

Other and more specific objects, features and advantages of the invention will appear from the detailed description given below, taken in connection with the accompanying drawings which form a part of this specification and illustrate by way of example one form of equipment which may be used in carrying out the invention. The invention consists in such novel features and combinations of features as may be hereinafter more specifically pointed out and specified in the appended claims.

In the drawings:

Fig. 1 is a side view, somewhat diagrammatic, of a supercalender equipped and arranged with steam showers and associated special equipment for carrying out the invention in the preferred way;

Fig. 2 is an enlarged transverse sectional view through one of the steam showers showing the preferred means by which the formaldehyde may be introduced into the steam showers; and

Fig. 3 is a longitudinal sectional view of portions of one of the steam showers.

Referring now to the drawings in further detail, the supercalender shown has ten superposed rolls as indicated at 10-19 inclusive, certain of the rolls having steel surfaces as indicated by the reference character S, and others having fiber surfaces of conventional type as indicated by the reference character F. So-called "fly rolls" are indicated at 20, 21 etc. for guiding the paper as it emerges from between the nip of adjacent rolls, into the next nip of the rolls. The paper may be fed as from a roll 22 onto the top roll of the calender and thence down through the calender onto a power-driven wind-up roll 23 of conventional form.

"Steam showers" are indicated at 24 and 25 for applying steam to the opposite surfaces respectively of the paper. It will be noted that each of these showers is so positioned as to apply steam to that surface of the paper which is about to be engaged successively by a plurality of steel rollers which act to iron out and polish the paper surface. That is, the steam shower 24 is positioned to apply steam to that surface of the paper which is to be engaged by the steel rollers 10 and 12, and the steam shower 25 applies steam to the surface of the paper which is to be engaged by steel rollers 15, 17 and 19.

As indicated in Fig. 2, the form of steam shower means here used may comprise central steam inlet pipes 30, 30' extending transversely of the moving web and having a slot or a series of apertures at 31 for permitting the steam to escape into an intermediate cylinder 32 surrounding the pipe 30. Steam and condensate escape through a slot or apertures at 33 on the lower side of the cylinder 32 and into an outer cylinder 34. Condensate drains from the latter cylinder through a conduit

35 running to waste, whereas the remaining steam passes up around between the walls of cylinders 32 and 34 to either a slot or a series of apertures 36 positioned along the top of the cylinder 34, and along a line transverse to the moving web closely adjacent thereto, so that a jet or jets of steam 37 forcefully impinge upon the paper web.

In order to embody the formaldehyde in the steam jet or jets 37, preferably a tank as at 40 is provided, connected by piping as at 41 to a pipe 42 extending longitudinally of the space between the cylinders 30' and 32. The lower side of pipe 42 is provided either with spaced apertures or a series of sprayers as at 42' (Fig. 3) permitting liquid to be sprayed out at a rate subject to regulation as hereinafter described onto the exterior of the pipe or cylinder 30' which is being maintained in heated condition by the presence of the steam. An aqueous 10-40% solution of the formaldehyde may be used in the tank 40. However, the percentage of the solution may be varied within wide limits.

At least the major part of the formaldehyde solution sprayed onto the heated exterior of the pipe or cylinder 30' is vaporized and thoroughly mixed with and carried along by the streams of steam through the orifice or apertures 36, and thus forcefully projected by the steam jet or jets 37 onto the paper web so that the steam, as it softens the coated paper surface, also insures that the formaldehyde will adequately penetrate the adhesive in the coating to impart moisture-proofing characteristics thereto. And since the paper web is immediately carried on between the nips of the calender rolls under substantial pressure, where the coating is also "ironed" and polished, the formaldehyde will promptly be locked or secured in place under pressure in the coating, insuring effective treatment of the coating and tending to prevent later escape of formaldehyde from the paper surface. With the formaldehyde incorporated in the coating in this way, it appears to continue to act on the coating while the paper is aging for some days or weeks to further enhance the waterproof and tough characteristics of the coating.

With this method of applying formaldehyde, the atmosphere surrounding the calender is surprisingly free of any escaping formaldehyde vapor, despite the immediate presence of high temperature steam which would normally be expected to cause the formaldehyde to be highly volatile and insure its distribution in the atmosphere. In fact the smell of formaldehyde was not objectionable around the calender rolls except at points closer than workmen would normally safely come. While the reasons for this unexpectedly desirable result are not fully understood, it is believed that as the steam escapes from the apertures at 36, its resulting expansion and consequent cooling in some manner causes the formaldehyde to be effectively retained against escape and to be carried along onto and into the web surface, either by reason of dissolving the gas in the fine particles of resulting condensate; or otherwise.

The draining of condensate from the bottom of the "steam showers" through pipes as at 35 will insure that the steam as it passes through the orifices at 36 will be substantially dry and free of droplets of water which would impart a non-uniform treatment to the web. At the same time any excess formaldehyde solution which is not substantially vaporized and entrained in the escaping steam, will be drained away through

the pipes 35. Thus the conventional steam shower construction is so used as to insure that both the steam and formaldehyde treatments on the web will be uniform.

It will be apparent that the invention may be applied to the treatment of paper board as well as paper and other webs, coated or uncoated, and which embody adhesives capable of being rendered moisture resistant by the action of formaldehyde.

It will be apparent that the expense for equipment for carrying out this method is small, since except for the formaldehyde mixing and regulating means hereinafter described, the preferred equipment essentially comprises the available 15 calenders or supercalenders and accompanying steam showers. While it is believed not to be essential that any special ventilating equipment or hoods be provided for confining or carrying away escaping vapor, if desired the upper surface of each steam shower may be provided with baffle plates or walls as at 45, 46 interconnected at their ends by properly shaped end pieces so as to provide a chamber 47, the top of which is substantially closed by the moving web. This structure 20 will tend to confine the steam and vapor for somewhat more effective treatment of the paper.

While the method is preferably carried out during the supercalendering operation where steam shower facilities are usually already available, it will be apparent that similar steam showers might be applied to the usual calender at the end of the paper making machine (which, of course, follows the usual dryer rolls of the machine) to permit the use of the invention at 35 that point if preferred, or in cases where supercalendering of the web may be unnecessary.

The temperature and amount of the steam used does not appear to be critical. Highly satisfactory results have been obtained using steam showers the same as customarily used in supercalendering coated paper. For example the steam entering the cylinder 30' may be at a temperature in the neighborhood of 255° F. and at a pressure of 60 lbs. The amount of formaldehyde in solution used is also not critical, although it is desirable that enough be used so that continuous sprays thereof will be directed onto the cylinder or pipe 30'. As above indicated, the percentage of formaldehyde used in the solution may also be varied within wide limits as only a small quantity is necessary in treating the coated paper for the above-indicated purposes, and any excess will be drained away in the condensate passing out through pipes 35.

The coated paper treated in accordance with this invention has been found to present a highly satisfactory surface with improved gloss for high speed lithographic printing, particularly for multi-colored printing.

One suitable form of regulating apparatus for supplying the formaldehyde solution will now be described in connection with the enlarged view thereof shown in Fig. 2 and a view thereof on a smaller scale in Fig. 1. The commercially available formaldehyde solution may be supplied as in a barrel 50, which is subjected to air pressure as by compressed air connection 51, the solution passing from the barrel through a shut-off valve 52 and a pipe 53, preferably having a check valve as at 54 at a point prior to its entry into the tank 40. Within or adjacent the tank 40 a mixing valve 55 of suitable known type may be provided for mixing the solution with a desired proportion of water coming in through a water

supply line 56 and a check valve 57. The mixing valve 55 may also be of a suitable float controlled type controlled in a known way as by a float 58 in the tank 40 and arranged so that whenever the level of the liquid in the tank is lower than a predetermined limit, the mixing valve will be opened to admit desired proportions of water and formaldehyde solution, but when the tank 40 is filled to a predetermined level, the mixing valve 55 will shut off the supplies of both the water and solution. The tank 40 is also preferably connected to an air pressure line as at 60 entering through a pressure regulating valve 61 having a vent pipe 62 which will be opened by the pressure regulating valve whenever the pressure in the tank 40 is greater than the pressure, as supplied by pipe 60 regulated by valve 61. The barrel 50, for example, may be subject to a pressure of 30 lbs. per square inch, whereas the tank 40 may normally be subjected to a pressure, for example, of 20 lbs. per square inch. Thus when the mixing valve 55 is opened by the float, the tank 40 will be subjected to pressure from the barrel high enough to allow the mixed liquids to enter, and sufficient air or vapor above the liquid in the tank 40 will escape through the vent 62 to allow the liquid level to rise to the desired predetermined point as controlled by the float.

The piping 41 for carrying the solution into the steam showers preferably is provided with a solenoid-operated shut-off valve 65 and the steam pipe 30 may also be provided with a similar valve 66, both these solenoid valves preferably being operable by the same circuit as indicated in Fig. 1 and arranged so that when the electric current is shut off, the flow of both solution and steam to the showers will be cut off.

As indicated in Fig. 1, the solution and steam may be carried to the shower 24 by branch pipe lines 41a and 30a respectively, which are connected to the piping 41 and the steam pipe 30.

While in the interests of economy in the use of formaldehyde, some special means is desirable for mixing the commercially available formaldehyde solution with water and for regulating the supply of the mixture properly under pressure, means other than that shown may, of course, be used such as mixing tanks from which the solution flows by gravity into the steam showers.

This application is a continuation-in-part of application Serial No. 143,185, filed February 9, 1950, now abandoned.

While the invention has been described in detail with respect to particular preferred examples, it will be understood by those skilled in the art after understanding the invention, that various changes may be made and equivalents may be used without departing from the spirit and scope of the invention.

What is claimed as new and desired to be secured by Letters Patent is:

1. In the calendering of a dried paper web which has been coated on the paper making machine with a mixture embodying clay and casein, the method of providing the dried web with a moisture-resistant hardened glossy print receptive surface suitable for high speed lithographic printing, which comprises forming an intimate intermixture of steam and formaldehyde, impinging said mixture in jet form onto a coated face of the dried coated web and immediately subjecting the thus treated face of the web to the ironing action of metal faced calender rolls until such face has been effectively calendered.

2. In the calendering of a dried paper web which has been coated with a mixture embodying clay and soya protein adhesive, the method of providing the dried web with a moisture-resistant glossy print receptive surface suitable for high speed lithographic printing, which comprises forming an intimate intermixture of steam and formaldehyde, impinging said mixture onto a coated face of the dried coated web and immediately subjecting the thus treated face of the web 10 to the ironing action of calender rolls until such face has been effectively calendered.

3. In the calendering of a dried paper web which has been coated with a mixture embodying

clay and an adhesive selected from the group consisting of casein and soya protein, the method of providing the dried web with a moisture-resistant glossy print receptive surface suitable for high speed lithographic printing, which comprises forming an intimate intermixture of steam and formaldehyde, impinging said mixture onto a coated face of the dried coated web and immediately subjecting the thus treated face of the web to the ironing action of calender rolls until such face has been effectively calendered.

RICHARD J. GRIMM.

No references cited.